# EUROPEAN PATENT SPECIFICATION

(11) **EP 0 450 722 B1**
(45) Date of publication and mention of the grant of the patent: **04.01.1995**
(21) Application number: 91200747.3
(22) Date of filing: 29.03.1991
(51) Int. Cl.: F02F 7/00, F02F 1/10

(54) **Process for obtaining a continuous metallurgical bond between the linings of the cylinders and the cast which constitutes the crankcase of an internal-combustion engine**
Verfahren für einen kontinuierlichen Metallbund zwischen Zylinderfutter und Kurbelgehäuseguss einer Brennkraftmaschine
Procédé pour obtenir une bondage métallurgique continue entre des fourreaux cylindres et un bâtiment-moteur moulé d'un moteur à combustion interne

(30) Priority: 06.04.1990 IT 1996890
(43) Date of publication of application: 09.10.1991
(73) Proprietor: ENIRISORSE S.p.A., I-00143 Roma (IT); ALUTEK S.r.l., I-10151 Torino (IT)
(72) Inventor: Guerriero, Renato, I-30175 Mestre-Venice (IT); Tangerini, Ilario, I-30175 Mestre-Venice (IT); Gallo, Sergio, I-10127 Turin (IT)
(74) Representative: Fusina, Gerolamo

(56) References cited:
- DE-A- 3 837 254
- FR-A- 1 340 869
- PATENT ABSTRACTS OF JAPAN vol. 11, no. 54 (M-563)(2501) 19 February 1987, & JP-A-61 215439 (YANMAR DIESEL ENGINE CO LTD) 25 September 1986
- PATENT ABSTRACTS OF JAPAN vol. 14, no. 113 (M-944)(4056) 02 March 1990, & JP-A-01 313652 (ISUZU MOTORS LTD) 19 December 1989
- PATENT ABSTRACTS OF JAPAN vol. 12, no. 145 (M-693)(2992) 06 May 1988, & JP-A-62 265453 (HONDA MOTOR CO LTD) 18 November 1987

## Description

The present invention relates to a process for obtaining a continuous metallurgical bond between the linings of the cylinders and the cast which constitutes the crankcase of an internal-combustion engine.

In an internal-combustion engine, each piston, made from an aluminum alloy, slides with precision inside a cylindrical hollow provided inside "the crankcase of the engine, which is generally made from cast iron, but which can also be obtained from a cast made from an aluminum alloy.

The precision of such a sliding is secured by segments or elastic piston rings made from steel or cast iron, arranged around the piston. In particular, in the crankcases made from aluminum alloys, the friction of the piston rings on the inner walls of the cylinder cause the latter to be worn and, over time, such a wear decreases the sliding precision, with the efficiency of the engine being consequently reduced.

In order to obviate this drawback, inside the hollow of the cylinders linings are inserted, which are made from high-wear-strength materials, such as, e.g., steel or other aluminum alloys.

These linings are inserted inside the engine crankcase, after the latter is manufactured by casting, by heat-fitting or, during the same casting step, arranging the linings as inserts inside the casting mold. In both cases, the coupling between the lining and the crankcase is achieved by mechanical gripping, without material continuity, and this may cause drawbacks in the cooling down of the internal surface of the cylinders by effect of poor heat conductivity due to the discontinuity between the materials. Furthermore, owing to such a discontinuity, and to the difference between the coefficience of heat expansion of the different materials, in the mean time, following repeated termal cycles, the adhesion and the mechanical hooking between the crankcase and the lining decreases, with said crankcase and lining consequently getting detached from each other and undergoing mutual movements, causing, due to the effect of insufficient cooling, a rapid decay of the quality of the internal lining surface finish.

It has been found that by means of a suitable surface treatment of the linings of the cylinders, a strong metallurgical bond can be obtained between said linings and the cast which constitutes the crankcase of an internal-combustion engine.

For example, JP-A-61215439 describes a process for obtaining a continuous metallurgical bond between the lining of the cylinders and the cast which constitutes the crankcase of an internal combustion engine, which crankcase is made of a meterial different from the material which constitutes the linings (the crankcase is made of an aluminium alloy and the linings is made of steel or the like annealed), comprising carrying out a surface treatment by depositing a thin nickel layer on the external surface of the lining and casting around the same lining the metal or metal alloy from which the crankcase is made. Therefore the metallurgical bond is obtained between aluminium and steel.

In particular, the process according to the present invention secures that the classic requirements of the welding operation are met: removal of surface impurities and oxides, intimate contact and coalescence of the materials to be bonded.

However, this type of welding is very different from other methods in that no external energy sources are required (e.g., heat, ultrasounds, and so forth) and the welding takes place during the course of the same casting.

Furthermore, metals which can be not easily coupled by means of other techniques can be bonded by means of such a welding type.

The Process according to the present invention for for obtaining a continuous metallurgical bond between the linings (2) of the cylinders, and the cast (1) which constitutes the crankcase of an internal-combustion engine, which crankcase is made of aluminum, or magnesium, or alloys of aluminum or magnesium and consists of a material different from the material which constitutes the linings (2), comprises the steps of:
carrying out a surface treatment by depositing a thin metal layer, said metal being different from the metals which are contained in the materials of the linings (2) and of the cast (1), said metal layer being able of increasing the wettability of, and the heat transfer coefficient between the materials of the lining (2) and of the cast (1),
and casting around the same lining (2), positioned inside the mould, the metal or alloys from which the crankcase is made,
characterised in that the lining (2) consists of aluminum, or magnesium, or of alloys of aluminum or magnesium, or of a composite material having aluminum, or magnesium, or alloys of aluminum or magnesium as its matrix, and in that the metal to be deposited on the external surface of the lining (2) is selected from among Au, Ag, Cu, Pt, Pd, Cr, W, Ir, Mo, Ta, Nb, Os, Re, Rh, Ru and Zr.

The lining may also be made from a composite material having as its metal matrix, aluminum or magnesium or aluminum or magnesium alloys: such a type of material is constituted by a metal phase (or a metal alloy phase), which surrounds and links other phases, which constitute the reinforcement (powders or ceramic fibres).

The reinforcement is endowed with high values of mechanical strength and hardness, and the stresses to which the matrix is submitted are transferred to it. The matrix, on the other hand, should be endowed with suitable characteristics as a function of the envisaged type of application.

The reinforcement can be constituted by long ceramic fibres or short ceramic fibres (Al₂O₃, SiC, Si₃N₄; BN, SiO₂) or by ceramic "whiskers" (SiC, Si₃N₄, B₄C, Al₂O₃) or by non-metal powders (SiC, BN, Si₃N₄, B₄C, Sio₂ or Al₂O₃).

The methods for preparing the composites can be the following:
- Dispersion of the reinforcement in the matrix on the molten state;
- Dispersion of the reinforcement in the matrix in a partially solid state;
- Powder metallurgy;
- Fiber metallurgy;
- Layer compacting;
- Infiltration.

The composite material can be obtained either directly or by means of a following mechanical machining/processing.

The metal which constitutes the thin layer, preferably having a thickness comprised within the range of from 10 to 100 nm, to be deposited onto the surface of the metal material or of the metal-matrix composite material, which should be different from those contained in the materials and in the cast, can be preferably selected from among Au, Ag, Cu, Pt, Pd, Cr, W, Ir, Mo, Ta, Nb, Os, Re, Rh, Ru and Zr.

The deposition of said thin metal layer can be preferably carried out by "sputtering" or by electrochemical deposition.

Also any other methods known in the art, of chemical, physical, and so forth, types, for surface coating can be used: for example, plasma-spraying, laser-assisted deposition, thermal-evaporation deposition, magneton-assisted deposition, CDV ("Chemical Vapour Deposition"), and so forth.

By using a suitable coating, the liquid to be cast will be capable of wetting the metal material or the metal-matrix composite to a sufficient extent to transfer heat to it, wash out the layer of oxide which is unavoidably formed on the surface of said material and directly binding to the material, in case a metal material is used, or to the metal matrix, if a composite is used.

Once that the material is adequately cleaned, coated and positioned inside the casting die, the casting operating parameters have to be so adjusted as to secure that a suitable stream of overheated liquid will lap the surfaces of the materials.

It is important that the position of the material inside the die is suitably selected and that the shape of the downward duct (ingress duct) and of the upward duct (egress duct) inside the die is properly designed, So that the liquid metal will be obliged to lap, wet and wash out the walls of the material before said liquid metal is cooled dawn to a too low temperature.

Hence, the matter is of keeping under control the following three parameters: material pre-heating temperature, metal (or alloy) casting temperature, flux conditions. In such a way, an excellent metallurgical bond between the material and the cast can be obtained.

The linings of the cylinders can be obtained by means of techniques known in the art (for example: gravity casting or pressure casting or die-casting or squeeze-casting; or powder metallurgy, or by infiltration or blending), and either directly or by a successive mechanical machining by tool machines or by plastic-working processes (such as extrusion, lamination or forging). Some examples are now given, which have the purpose of better illustrating the invention, but which no way should be construed as being limitative of the same invention:

### EXAMPLE 1

### (Laboratory test)

- The lining is constituted by a tube made from a hypereutectic alloy of Al-Si with a content of 17% of Si, with an outer diameter of 50 mm, a thickness of 5 mm and a height of 65 mm, obtained by gravity casting.
- The outer surface of the lining is coated by sputtering with a thin gold layer.
- The material which constitutes the cast is an Al-Si alloy with a content of 9% of Si.
- The casting die is made of graphite (see the Figure) wherein:
   (1) is the graphite die,
   (2) is the lining, and
   (3) is the casting channel.
- The lining and the die are pre-heated at 350°C.
- The temperature of the metal of the cast is of 700°C.
- The volume of cast material is of approximately 400 cm³.
- The casting is carried out in by bottom casting.

### EXAMPLE 2

### (Laboratory test)

- The lining is constituted by a tube made from a composite material with an outer diameter of 50 mm, a thickness of 5 mm and a height of 65 mm, obtained by gravity casting.
- The composite material, obtained by infiltration, is constituted by a matrix of an eutectic Al-Si alloy, with a content of 13% of Si, and with a reinforcement constituted by an SiC powder at 55% by volume (average diameter of powder particles: 20 µm).
- The outer surface of the lining is coated by sputtering with a thin gold layer.
- The material which constitutes the cast is an Al-Si alloy with a content of 9% of Si.
- The casting die is made of graphite (see the Figure), as in Example 1
- The lining and the die are pre-heated at 300°C.
- The temperature of the metal of the cast is of 650°C.
- The volume of cast material is of approximately 400 cm³.
- The casting is carried out by bottom casting

### EXAMPLE 3

### (Industrial Test)

- The test was carried out on an industrial facility for casting crankcases for four-cylinder engines.
- The linings, obtained by extrusion, are constituted by tubes made from a composite material, with an outer diameter of approximately 95 mm, a thickness of about 5 mm and a height of about 130 mm.
- The composite material, obtained by infiltration and dilution, is constituted by a matrix of an eutectic Al-Si alloy, with a content of 13% of Si, and with a reinforcement constituted by an SiC powder at 25% by volume (average diameter of the powder 20 µm).
- The outer surface of the lining is coated by sputtering with a thin gold layer.
- The material which constitutes the cast is an Al-Si alloy with a content of 9% of Si.
- The industrial casting die is made of cast iron.
- The linings are preheated at 300°C.
- The temperature of the cast metal is of about 700°C.
- The volume of cast material is of approximately 10 dm³.
- The casting is carried out by bottom casting.

### EXAMPLE 4

### (Industrial Test)

- The test was carried out on an industrial facility for casting crankcases for four-cylinder engines.
- The linings, obtained by extrusion, are constituted by tubes made from a composite material, with an outer diameter of approximately 95 mm, a thickness of about 5 mm and a height of about 130 mm.
- The composite material, obtained by mixing, is constituted by a matrix of an eutectic Al-Si alloy, with a content of 9% of Si, and with a reinforcement constituted by an SiC powder at 15% by volume (average diameter of the powder 20µm).
- The outer surface of the lining is coated by sputtering with a thin gold layer.
- The material which constitutes the cast is an Al-Si alloy with a content of 9% of Si.
- The industrial casting die is made of cast iron.
- The linings are pre-heated at 300°C.
- The die is preheated at about 370°C.
- The temperature of the cast metal is of about 700°C.
- The volume of cast material is of approximately 10 dm³.
- The casting is carried out by bottom casting.

## Claims

1. Process for obtaining a continuous metallurgical bond between the linings (2) of the cylinders, and the cast (1) which constitutes the crankcase of an internal-combustion engine, which crankcase is made of aluminum, or magnesium, or alloys of aluminum or magnesium and consists of a material different from the material which constitutes the linings (2), said process comprising the steps of:
carrying out a surface treatment by depositing a thin metal layer, said metal being different from the metals which are contained in the materials of the linings (2) and of the cast (1), said metal layer being able of increasing the wettability of, and the heat transfer coefficient between the materials of the lining (2) and of the cast (1),
and casting around the same lining (2), positioned inside the mould, the metal or alloys from which the crankcase is made,
characterised in that the lining (2) consists of aluminum, or magnesium, or of alloys of aluminum or magnesium, or of a composite material having aluminum, or magnesium, or alloys of aluminum or magnesium as its matrix, and in that the metal to be deposited on the external surface of the lining (2) is selected from among Au, Ag, Cu, Pt, Pd, Cr, W, Ir, Mo, Ta, Nb, Os, Re, Rh, Ru and Zr.

2. Process according to claim 1, characterised in that the lining (2) consists of a composite material containing non-metal powders selected from among SiC, BN, Si₃N₄, B₄C, SiO₂ or Al₂O₃, as its reinforcement.

3. Process according to claim 1, characterised in that the lining (2) consists of a composite material having ceramic whiskers selected from among SiC, Si₃N₄, B₄C, SiO₂ or Al₂O₃, as its reinforcement.

4. Process according to claim 1, characterised in that the lining (2) consists of a composite material having long or short ceramic fibres selected from among SiC, BN, Si₃N₄, B₄C, SiO₂ or Al₂O₃, as its reinforcement.

5. Process according to claims 2, 3, and 4 characterised in that the lining (2) consists of a composite material containing powders, whiskers or long or short ceramic fibres, in a concentration of from 10 to 60 % by volume, as its reinforcement.

6. Process according to claim 1, characterised in that the deposition of a thin layer of metal takes place by sputtering.

7. Process according to claim 1, characterised in that the deposition of a thin layer of metal takes place by electrochemical deposition.

8. Process according to claim 1, characterised in that the deposition of a thin layer of metal takes place by chemical deposition.

9. Process according to claim 1 characterised in that the deposition of a thin layer of metal takes place by plasma-spraying or by thermal evaporation or by CVD (Chemical Vapor Deposition), or by a laser-assisted or magnetron-assisted deposition technology.

10. Process according to claim 1, characterised in that the lining (2) is obtained by gravity-casting, pressure-casting, die-casting, or squeeze-casting, or by powder metallurgy or by infiltration or blending, either directly or with successive machanical tool-machining, or mechanical plastic processing, such as extrusion, lamination or forging.

11. Process according to claim 1, characterised in that the composite material is obtained by dispersing the reinforcement in the matrix in the molten state, or by dispersing the reinforcement in the matrix in a partially solid state, or by powder metallurgy, or by metal-casting the fibres, or by layer-compacting, or infiltration.

12. Process according to claim 1, characterised in that the thin metal layer deposited on the outer surface of the lining (2) is comprised within the range of from 10 nm to 100 nm.

## Patentansprüche

1. Verfahren zum Herstellen eines kontinuierlichen Metallbundes zwischen dem Zylinderfutter (2) und dem Kurbelgehäusegußteil (1) einer Brennkraftmaschine, wobei das Kurbelgehäuse aus Aluminium oder Magnesium oder aus Legierungen von Aluminium oder Magnesium hergestellt ist und aus einem gegenüber dem das Futter (2) bildenden Material verschiedenen Material ist, mit den folgenden Verfahrensschritten:
Oberflächenbehandlung durch Auftragen einer dünnen Metallschicht, wobei das Metall sich von den Metallen unterscheidet, die in den Materialien des Futters (2) oder des Gußteils (1) enthalten sind, wobei die Metallschicht zur Erhöhung der Benetzbarkeit der Materialien und des Wärmeleitkoeffizienten zwischen den Materialien des Futters (2) und des Gußteils (1) geeignet ist, und
Gießen des Metalls oder der Legierungen, aus dem das Kurbelgehäuse besteht, um das gleiche Futter (2) das innerhalb der Form angeordnet ist,
dadurch gekennzeichnet, daß das Futter (2) aus Aluminium oder Magnesium oder aus Legierungen von Aluminium oder Magnesium oder aus einem Verbundmaterial mit Aluminium oder Magnesium oder Legierungen von Aluminium oder Magnesium als Matrix besteht und daß das auf der Außenfläche des Futters (2) aufzutragende Metall aus Au, Ag, Cu, Pt, Pd, Cr, W, Ir, Mo, Ta, Nb, Os, Re, Rh, Ru und/oder Zr ausgewählt ist.

2. Verfahren nach Anspruch 1, dadurch gekennzeichnet, daß das Futter (2) aus einem Verbundmaterial besteht, das zur Verstärkung nicht-metallische Pulver ausgewählt aus SiC, BN, Si₃N₄, B₄C, SiO₂ oder Al₂O₃ enthält.

3. Verfahren nach Anspruch 1, dadurch gekennzeichnet, daß das Futter (2) aus einem Verbundmaterial besteht, das zur Verstärkung Whisker ausgewählt aus SiC, Si₃N₄, B₄C, SiO₂ oder Al₂O₃ enthält.

4. Verfahren nach Anspruch 1, dadurch gekennzeichnet, daß das Futter (2) aus einem Verbundmaterial besteht, das zur Verstärkung lange oder kurze Keramikfasern ausgewählt aus SiC, BN, Si₃N₄, B₄C, SiO₂ oder Al₂O₃ enthält.

5. Verfahren nach Anspruch 2, 3 oder 4, dadurch gekennzeichnet, daß das Futter (2) aus einem Verbundmaterial besteht, das zur Verstärkung Pulver, Whisker oder lange oder kurze Keramikfasern in einer Konzentration von 10 bis 60 Vol.-% enthält.

6. Verfahren nach Anspruch 1, dadurch gekennzeichnet, daß das Auftragen einer dünnen Metallschicht durch Sputtern erfolgt.

7. Verfahren nach Anspruch 1, dadurch gekennzeichnet, daß der Auftrag einer dünnen Metallschicht durch elektrochemische Abscheidung erfolgt.

8. Verfahren nach Anspruch 1, dadurch gekennzeichnet, daß der Auftrag einer dünnen Metallschicht durch chemische Abscheidung erfolgt.

9. Verfahren nach Anspruch 1, dadurch gekennzeichnet, daß der Auftrag einer dünnen Metallschicht durch Plasmasprühen, durch thermisches Aufdampfen, durch chemische Abscheidung aus der Dampfphase (CVD) oder durch Laserunterstütztes oder Magnetron-unterstütztes Abscheiden erfolgt.

10. Verfahren nach Anspruch 1, dadurch gekennzeichnet, daß das Futter (2) erhalten wird durch Gravitationsguß, Preßguß, Druckguß, Formdruckguß, Pulvermetallurgie, Infiltration oder Vermischen entweder direkt oder mit anschließender mechanischer Werkzeugbearbeitung, oder durch mechanische, plastische Verarbeitung, wie Extrusion, Lamination oder Warmmassivumformung erfolgt.

11. Verfahren nach Anspruch 1, dadurch gekennzeichnet, daß das Verbundmaterial erhalten wird durch Dispergieren des Verstärkungsmaterials in der Matrix im geschmolzenen Zustand oder durch Dispergieren der Verstärkung in der Matrix in teilweise festem Zustand, durch Pulvermetallurgie, durch Metallbeschichtung der Fasern, durch Schichtverdichtung oder durch Infiltration.

12. Verfahren nach Anspruch 1, dadurch gekennzeichnet, daß die dünne Metallschicht, die auf der Außenfläche des Futters (2) aufgetragen ist, im Bereich von 10 nm bis 100 nm beträgt.

## Revendications

1. Procédé pour obtenir une liaison métallurgique continue de chemises (2) de cylindres, et la pièce moulée (1) qui constitue le carter d'un moteur à combustion interne, ledit carter étant fabriqué en aluminium ou en magnésium, ou en alliages d'aluminium ou de magnésium et constitué d'un matériau différent du matériau constituant les chemises (2), ledit procédé comprenant les étapes de :
mise en oeuvre d'un traitement de surface par dépôt d'une fine couche de métal, ledit métal étant diffèrent des métaux contenus dans les matériaux des chemises (2) et de la pièce moulée (1), ladite couche de métal étant susceptible d'augmenter la mouillabilité des matériaux des chemises (2) et de la pièce moulée (1) et le coefficient de transfert de chaleur entre ces dits matériaux.
et le moulage autour desdites chemises (2) placées à l'intérieur du moule, du métal ou des alliages qui constituent le carter,
caractérisé par le fait que chaque chemise (2) est constituée d'aluminium ou de magnésium, ou d'alliages d'aluminium ou de magnésium, ou d'un matériau composite ayant pour matrice de l'aluminium ou de magnésium, ou des alliages d'aluminium ou de magnésium et par le fait que le métal devant être déposé sur la surface externe des chemises (2) est choisi parmi Au, Ag, Cu, Pt, Pd, Cr, W, Ir, Mo, Ta, Nb, Os, Re, Rh, Ru et Zr.

2. Procédé selon la revendication 1, caractérisé par le fait que les chemises (2) sont constituées d'un matériau composite contenant des poudres non métalliques choisies parmi SiC, BN, Si₃N₄, B₄C, SiO₂ ou Al₂O₃ comme renforcement.

3. Procédé selon la revendication 1, caractérisé par le fait que les chemises (2) sont constituées d'un matériau composite ayant des trichites céramiques choisis parmi SiC, Si₃N₄, B₄C, SiO₂ ou Al₂O₃ comme renforcement.

4. Procédé selon la revendication 1, caractérisé par le fait que les chemises (2) sont constituées d'un matériau composite ayant des fibres céramiques courtes ou longues choisies parmi SiC, BN, Si₃N₄, B₄C, SiO₂ ou Al₂O₃ comme renforcement.

5. Procédé selon la revendication 2, 3 et 4 caractérisé par le fait que les chemises (2) sont constituées d'un matériau composite contenant des poudres, des trichites ou des libres céramiques courtes ou longues, dans une concentration de 10 à 60% en volume comme renforcement.

6. Procédé selon la revendication 1, caractérisé par le fait que le dépôt de la fine couche de métal a lieu par pulvérisation.

7. Procédé selon la revendication 1, caractérisé par le fait que le dépôt de la fine couche de métal a lieu par dépôt électrochimique.

8. Procédé selon la revendication 1, caractérisé par le fait que le dépôt de la fine couche de métal a lieu par dépôt chimique.

9. Procédé selon la revendication 1, caractérisé par le fait que le dépôt de la fine couche de métal a lieu par pulvérisation de plasma ou par évaporation thermique ou par CVD (dépôt chimique en phase vapeur), ou selon une technique de dépôt assistée par laser ou assistée par magnétron.

10. Procédé selon la revendication 1, caractérisé par le fait que les chemises (2) sont obtenues par coulage, moulage sous pression, coulée en coquille, ou moulage par compression, ou par métallurgie des poudres ou par infiltration ou par mélange, soit directement avec usinages mécaniques successifs, ou avec traitement mécanique plastique tel que extrusion, laminage ou forgeage.

11. Procédé selon la revendication 1, caractérisé par le fait que le matériau composite est obtenu par dispersion du renforcement dans la matrice à l'état fondu, ou par dispersion du renforcement dans la matrice dans un état partiellement solide, ou par métallurgie des poudres ou par revêtement métallique des fibres, ou par compactage des couches, ou par infiltration.

12. Procédé selon la revendication 1, caractérisé par le fait que la fine couche métallique déposée sur la surface externe des chemise (2) est comprise dans un domaine de 10 nm à 100 nm.
